

## UNITED STATES PATENT OFFICE

2,198,777

## HARD BITUMINOUS MATERIAL

Kenneth C. Laughlin, Baton Rouge, La., assignor  
to Standard Oil Development Company, a cor-  
poration of Delaware

No Drawing. Application March 31, 1936,  
Serial No. 71,925

1 Claim. (Cl. 196—152)

This invention relates to hard bituminous material and a process for preparing the same. More particularly it relates to high melting asphalts having a definite change in penetration with temperature and being especially suitable for the manufacture of molded asphaltic products generally and electric storage battery box compound specifically. The invention will be fully understood from the following description.

10 Asphalts may be obtained from petroleum in a variety of different ways. The particular method used depends very largely upon the use to which the asphalt is to be put. Asphalts to be used for electric storage battery box compound 15 and molded asphaltic products generally must meet certain specifications defined by the manufacturers of such products. These specifications are met at the present time by compounding natural asphalt (Gilsonite) with various petroleum asphalts. These asphalt blends are unsatisfactory for battery box manufacture in some respects and the manufacturers have drawn up a set of specifications for an ideal bitumen to be used in compounding battery boxes.

20 Thus an asphalt to be used for battery box compound should have a penetration between 14 and 18 at 150° F./100 grams/5 secs. as determined by Test No. D5-25 of the American Society for Testing Materials (A. S. T. M.).

25 The susceptibility factor should be between 27 and 35 as calculated by the following formula:

$$10 \times \frac{\text{Penetration} @ 150^\circ \text{F}/100\text{g}/5 \text{secs.}}{\text{Penetration} @ 115^\circ \text{F}/200\text{g}/5 \text{secs.}} + \frac{\text{Penetration} @ 185^\circ \text{F}/50\text{g}/5 \text{secs.}}{\text{Penetration} @ 150^\circ \text{F}/100\text{g}/5 \text{secs.}}$$

30 The softening point should be above about 260° F. as determined by the ring and ball method, Test No. D86-26 of the A. S. T. M.

35 The ductility should be high, that is about 35 to 40 centimeters at 185° F. at the rate of 5 cm./min. as determined by Test No. D113-35 of the A. S. T. M.

The present invention is directed to a new process for obtaining from petroleum, asphalts having the above characteristics.

40 It is already known that asphalt may be precipitated from petroleum and fractions thereof by diluting the same with liquefied normally gaseous hydrocarbons at normal or slightly higher temperatures. It has been found, however, that the asphalts so produced do not have the required penetration, susceptibility and ductility characteristics to adapt them for use as battery box compound and molded asphaltic products.

45 It has now been found that if a petroleum residue is diluted with a liquefied hydrocarbon having 4 carbon atoms and the mixture heated to a high temperature, the asphalt so precipitated will have the desired characteristics referred to above. In effect this method may be said to consist in the high temperature butane precipitation

of asphalt from petroleum. The method is carried out as follows:

A petroleum residue containing asphalt is mixed with from 4 to 10, preferably about 6 to 8, volumes of liquefied butane. Other hydrocarbons having 4 carbon atoms such as isobutane, butylene, and isobutylene may, of course, also be used. The mixture is heated to a temperature between 150 and 300° F., preferably about 200° F., and pressure is maintained sufficient to 10 retain the butane in liquid phase at the temperature of working. The mixture is allowed to stand at substantially the same high temperature until the asphaltic layer has settled out and it is then drawn off. It is found that the asphalt 15 when so precipitated comes down in a fluid condition which greatly facilitates efficient mixing and settling.

It will be understood that the precipitation may be carried out in a batch manner as indicated above, or in a continuous counter-current manner either in a tower or in a series of separate but inter-connected stages. The apparatus for the counter-current treating may be substantially the same as that usually employed in such processes, but special provision must, of course, be made for heating the mixture and it is preferable to insulate the settling chamber to prevent undue heat losses.

The following example illustrates the application of the process:

A Lago (Venezuela) crude petroleum is distilled to about 47.5% bottoms having a penetration of 180 to 200 at 77° F./100g/secs. The bottoms is mixed with about 7 volumes of butane and the mixture heated to a temperature of about 200° F. where it is maintained until the precipitated asphalt has settled. The asphalt layer which is liquid is drawn off and the butane is stripped therefrom with natural gas at a temperature of about 400° F. The asphalt so obtained has the following characteristics:

|                                      |          |         |
|--------------------------------------|----------|---------|
| Yield on bottoms                     | per cent | 40      |
| Softening point (ball and ring), °F. |          | 263     |
| Flash point, Cleveland O. C., °F.    |          | 560 45  |
| Ductility @ 150° F., 5 cm./min.      |          | 9       |
| Ductility @ 185° F., 5 cm./min.      |          | 38      |
| Susceptibility factor                |          | 33.7    |
| Penetration @ 77° F./100g./5 sec.    |          | 0       |
| Penetration @ 115° F./200g./5 sec.   |          | 11 50   |
| Penetration @ 150° F./100g./5 sec.   |          | 17.5    |
| Penetration @ 185° F./50g./5 sec.    |          | 31      |
| Soluble in CS <sub>2</sub>           |          | 99.80   |
| Insoluble in 86° naphtha             |          | 77.2    |
| Fixed carbon                         |          | 36.2 55 |
| Specific gravity @ 77° F.            |          | 1.006   |
| Volatile 5 hrs. @ 500° F. 50 grams   |          | 0.96    |

The fixed carbon was determined by the following:

